

## UNITED STATES PATENT OFFICE

JOSEPH H. CHEETHAM, OF DECATUR, ILLINOIS, ASSIGNOR TO MUELLER CO., OF DECATUR, ILLINOIS, A CORPORATION OF ILLINOIS

## WHITE BRONZE

No Drawing.

Application filed April 16, 1929. Serial No. 355,671.

The present invention relates to an alloy adapted for various commercial purposes and which will be superior to bronze, although possessing most of its valuable characteristics.

The alloy is particularly useful in the manufacture of bath room and plumbing articles, but is not limited to such applications, since it can be employed to take the place of the so-called white brass, German silver, and Monel metal, as well as many other commercial alloys sold under various trade names.

The alloy is characterized by possessing a color which is whiter than the well known nickel plate, and has been found under test to resist corrosion in the atmosphere, salt water spray, fumes and gases, as well as acids commonly found in the lavatories and water supply systems. The metal under such tests has been found to be superior to any of the usual alloys employed for this purpose.

Heretofore, with most alloys it has been necessary to cast with the greatest care, and expert workmanship, as well as costly machinery and processes, have been necessary.

With the present alloy, the usual brass castings and cores may be employed, and no special moulding conditions are necessary. In other words, regular brass moulds are satisfactory, a particularly coarse sand is not required, and usual aggravating moulding conditions such as venting to exit gases is eliminated.

Moreover, the melting conditions do not require any special attention, it being possible to melt the alloy in a large furnace in batches of one thousand pounds (1000 lbs.) or less, whereas with many alloys melts over one hundred and fifty pounds (150 lbs.) have been impracticable, due to the rapidity of the metal cooling below pouring temperature.

The present alloy possesses physical qualities which will be later described, which enable it to be machined at the same speeds and feeds as regular brass or bronze, and on the same machines with identical tools.

An important feature of the invention resides in its property of permitting polishing and buffing with the same ease customary with common brass or bronze. The luster is

long wearing, and under careful tests, has surpassed nickel and chromium plating. If for any reason, after a long interval, a dullness appears, ordinary household cleaning compounds can be employed to restore the finish, and if the article formed of my improved alloy is kept cleaned with soap and water at regular intervals, there will be no tarnish or dullness as the metal is solid all the way through.

I have found that this improved alloy is slightly tougher than common bronzes, has equal elasticity and elongation when stretched and substantially the same hardness. A comparsion of a test is given below:

|                  | White<br>bronze | Red<br>bronze |
|------------------|-----------------|---------------|
| Tensile strength | 32,000          | 30,000        |
| Elastic limit    | 26,000          | 22,000        |
| Elongation in 2" | 10%             | 20%           |
| Brinell hardness | 58%             | 53%           |

The composition of my improved alloy is as follows:

|           |     |    |       |    |
|-----------|-----|----|-------|----|
| Copper    | 50  | to | 58%   | 76 |
| Tin       | 0.5 | to | 3%    |    |
| Zinc      | 12  | to | 20%   |    |
| Iron      | 0.0 | to | 0.75% |    |
| Nickel    | 12  | to | 19%   |    |
| Manganese | 0.0 | to | 0.5%  |    |
| Lead      | 8   | to | 13%   | 80 |

I have found that an alloy prepared with ingredients in the following proportions will also be quite satisfactory:

|           |     |    |       |    |
|-----------|-----|----|-------|----|
| Copper    | 52  | to | 55%   | 85 |
| Tin       | 1.5 | to | 2.5%  |    |
| Lead      | 10  | to | 12%   |    |
| Zinc      | 15  | to | 19%   |    |
| Iron      | 0.0 | to | 0.75% | 90 |
| Nickel    | 15  | to | 18%   |    |
| Manganese | 0.0 | to | 0.25% |    |

It will be observed that traces of manganese and iron are employed. In most cases, the iron is present in the copper, since it is impossible to obtain a pure copper, and the manganese is added in order to suspend the iron in a matrix of copper.

I have found that with any alloy containing over 58% copper, tarnishing will develop

under mild acids and from exposure to the atmosphere. I have also determined that iron is a detriment to the metal, but cannot be eliminated, since, as stated, the purest and best copper obtainable contains a small percent of iron. For this reason, manganese is added, since the copper without the addition of the manganese would repulse the iron, and allow it to collect in large quantities throughout the mass, resulting in ruining tools when the material is being machined and in the case of pressure castings causing leakage.

Lead, as is well known, materially aids machining, but also repulses copper when in the molten state, and unless thoroughly amalgamated, produces lumps of lead segregated from the copper, generally called "lead swets". For this reason, tin is employed to amalgamate the lead, since tin has an affinity for lead and copper, and the addition of a small percentage of tin up to 3% amalgamates the lead with the other elements, and the combination produces a homogeneous metal with the added advantages of maintaining for indefinite periods its silver-like luster. The addition of the lead acts to whiten the copper.

Zinc is used as a flux and cleaner for the copper, and materially aids foundry conditions. Its use with lead, moreover, cheapens the mixture and permits the production of a less expensive but superior alloy to many of those now in use.

As stated, no special furnaces or processes are necessary, since the melting is quite in accordance with that followed for commercial brasses and bronzes. This is a feature not heretofore possible with most of the commercially usable alloys.

As far as fluxes are concerned, no special material is required, and this should be carefully observed, since it is the special melting and special furnaces, as well as small melts and accurate proportions of fluxes which render present commercial alloys so expensive and oft-times inefficient and unsatisfactory.

The use of lead from 8% to 13% is very important, since in many of the commercial alloys which have come to my attention the failure to appreciate properly the value and use of this ingredient has rendered a particular alloy ruinous.

The present invention has a close resemblance in physical characteristics to commercial bronzes, and for the purpose of laboratory and plumbing fixtures and articles, is both cheaper and more commercially reliable than those heretofore used.

The proportions above given have all been found satisfactory, and if followed with reasonable care and skill will produce a white bronze of superior quality which will be more advantageous than so-called nickel or chro-

mium plating and many well known commercial products.

In the appended claim, it will be understood that equivalents and slight alterations in the quantity and nature of the ingredients is considered to be covered within the scope of the appended claim.

I claim:

An alloy of the class described comprising copper 52 to 55%, tin 1.5 to 2.5%, lead 10 to 12%, zinc 15 to 19%, nickel 15 to 18%, iron in substantial amounts up to 0.75% and manganese in substantial amounts up to 0.25%.

In testimony whereof I have hereunto set my hand.

JOSEPH H. CHEETHAM.

80

85

90

95

100

105

110

115

120

125

130